

## UNITED STATES PATENT OFFICE

ALFRED CLAUDE JESSUP, OF CLAMART, FRANCE

## PROCESS FOR THE MANUFACTURE OF MAGNESIUM

No Drawing. Application filed May 18, 1930, Serial No. 453,865, and in Germany June 1, 1930.

It is a known fact that in the electrolytic manufacture of magnesium from magnesium chloride, that on the one hand, the electrolytic yield of the operation, that is, the amount of magnesium obtained per unit quantity of electric current, will rapidly diminish when the magnesium chloride contains traces of water, and on the other hand, the complete drying of magnesium chloride is a very difficult expensive operation.

It has been further observed that a mixture of potassium chloride and magnesium chloride in the proportion of two or three molecules of the first to one molecule of the second, may be treated by electrolysis with a satisfactory efficiency, even if it contains 1 to 2 per cent of water, but this efficiency will gradually diminish when the molecular proportion of potassium chloride to the magnesium chloride exceeds 3 to 1, the percentage of water remaining within the above-mentioned limits. On the contrary, with the latter mixture, a very good yield is obtained when the percentage of water is below 1 per cent.

The present invention has for its object to obviate the drawbacks specified in the first paragraph, and to utilize the remarkable effects above mentioned.

For this purpose, there is prepared in the first place an incompletely dehydrated mixture of potassium chloride and magnesium chloride, in the proportion of three molecules of the first-mentioned chloride for at least one molecule of the second, and this mixture is treated by electrolysis until the proportion of potassium chloride exceeds three molecules for one molecule of magnesium chloride, due to the precipitation of the magnesium. The greater part of the water contained in this mixture has now been eliminated. The said mixture, which is practically anhydrous, is then subjected to a second electrolysis and this is effected with an excellent yield.

It is observed that the quantity of electric current consumed during these two electrolytic treatments is less than the quantity which would have been consumed in the first place during a preliminary heating of the

mixture in order that it will be completely dehydrated, and less than the amount which would have been used during an efficient electrolysis of the dry mixture.

It is advantageous to effect the two electrolytic treatments in two different tanks or vats, and in this manner, a vat which is employed for the first electrolysis will serve to supply several vats used for the second electrolysis.

The mixture used in the first electrolysis is preferably dehydrated in part, by one or the other of the following processes.

1. By adding, in the hydrated state, magnesium chloride or a mixture of magnesium chloride and potassium chloride, or carnallite, in a gradual manner and in relatively small quantities to a relatively large liquid mass of magnesium chloride or a mixture of dehydrated magnesium chloride and potassium chloride, as specified in the pending U. S. application No. 440,637 dated March 31, 1930 in the name of Madame Eliza Lacell, entitled: Process for the dehydration of carnallite and particularly of magnesium chloride.

2. By adding, during the drying of magnesium chloride, potassium chloride obtained from the second electrolysis, in such manner that the potassium chloride will follow a closed circuit and will not exceed the percentage desired for the first electrolyte as specified in the pending application filed in U. S. A. by P. Camescasse, on behalf of The Magnesium Production Co. Ltd. on April 14, 1930, entitled: Improvements in process for the manufacture of magnesium, Serial No. 444,236.

Herein, the vat employed for the first electrolysis is disposed between the melting vat and the vat employed for the final electrolysis. Before the said mixture reaches this latter vat, the water will be eliminated.

I claim:

1. Process for the production of magnesium by electrolysis, consisting in first preparing a mixture of potassium chloride and magnesium chloride containing less than three molecules of the former to one of the latter, and containing not substantially more

than 2% of water; proceeding with a first electrolysis of the mentioned mixture in such a way as to obtain a mixture which is practically anhydrous and containing more than 5 three molecules of potassium chloride for one of magnesium chloride, and then to proceed with a second electrolysis of the mixture obtained as a result of the first electrolysis.

2. Process according to claim 1 in which 10 the mixture obtained at the end of the first electrolysis is conveyed into a separate electrolytic apparatus for the second electrolysis.

3. Process according to claim 1 in which 15 the mixture obtained at the end of the first electrolysis is distributed among a plurality of electrolytic cells for carrying out the second electrolysis.

4. Process for the production of magnesium by electrolysis, consisting in gradually adding small masses containing, at least partially hydrated magnesium chloride, to a large mass containing substantially anhydrous magnesium chloride, one at least of 25 said materials containing potassium chloride, so as to obtain a mixture of potassium chloride and magnesium chloride containing less than three molecules of the first to one of the second and, at the most, 2% of water; proceeding with a first electrolysis of the named 30 mixture so as to obtain a mixture which is practically anhydrous and containing more than three molecules of potassium chloride to one of magnesium chloride; and then proceeding with a second electrolysis of the 35 mixture obtained from the first electrolysis.

5. Process for the production of magnesium by electrolysis, consisting in adding, during the dehydration at the latest, magnesium chloride, potassium chloride, coming from the second electrolysis described above, in such amounts as to obtain a mixture of potassium chloride and magnesium chloride containing less than three molecules of the 45 first to one of the second and at the most 2% water; then proceeding with a first electrolysis of the aforesaid mixture so as to obtain a practically complete dehydration, and to form an electrolyte containing at least three 50 molecules of potassium chloride to one of magnesium chloride; and then proceeding with a second electrolysis of the mixture obtained from the first electrolysis, and introducing at least in part, the mixture remaining 55 at the end of the second electrolysis, into the process of dehydration of the magnesium chloride constituting the first stage of the 60 process.

6. A process for the electrolytic manufacture of magnesium which comprises first preparing an incompletely dehydrated mixture of potassium chloride and magnesium chloride in the proportion of two to three molecules of the former to one of the latter; subjecting such mixture, in a molten state to a

first electrolysis in order to obtain a mixture containing at least three molecules of potassium chloride to one molecule of magnesium chloride which is substantially anhydrous, and subjecting such mixture which is thus practically dehydrated, to a second electrolysis.

In testimony whereof I have signed this specification.

ALFRED CLAUDE JESSUP. 75

80

85

90

95

100

105

110

115

120

125

130